

Oct. 31, 1939.

W. MEYER

2,177,735

LUMINOUS BODY

Filed Aug. 4, 1937



INVENTOR  
Wilfried Meyer  
BY Harry E. Dunham  
ATTORNEY

## UNITED STATES PATENT OFFICE

2,177,735

## LUMINOUS BODY

Wilfried Meyer, Birkenwerder, near Berlin, Germany, assignor to General Electric Company, a corporation of New York

Application August 4, 1937, Serial No. 157,424  
In Germany August 12, 1936

## 4 Claims. (Cl. 176—1)

My invention relates to improvements in luminous bodies adapted when acted upon by electrons or ultraviolet rays to emit light.

There are a large number of substances which when acted upon by light of short wave length or by electrons are made luminous. Such substances are used for example in the manufacture of luminous screens in Braun tubes. It is known that the radiation caused by the action of electrons is so much the stronger the higher the velocity of the electrons. However, a difficulty is caused by the fact that most of the luminous substances such for example as zinc silicate or cadmium silicate containing oxides of heavy metals such as manganese oxide are non-conductive. When such substances are impinged upon by electrons they are charged thus producing an electric counterfield. Thus the intensity of the radiation is reduced. Where the velocity of the electrons is small their energy may not even be sufficient to excite luminescence of the substances, because the action of the active field on the electrons is nearly compensated by the action of the retarding field. To avoid this the luminous substances are applied to the conductive screen in layers which are as thin as possible, in order to reduce the resistance opposed to the flow of the electrons from the screen. However, the particles of the luminous screen make contact with their carrier only at some points, and a luminous grain presents a very small cross-section for transmitting the electrons to the metal.

The object of the improvements is to provide a luminous body in which the luminous substance is in large surface contact with the conductive carrier and thus to produce luminous screens which have strong radiation also in case of low velocity of the electrons. With this object in view my invention consists in manufacturing the carrier of the luminous substance from compounds, and preferably from oxides, the metallic components of which simultaneously are parts of the luminous coating, the said luminous coating being produced on the said conductive carrier by chemical transformation of the surface, for example by transformation in a solid state.

For the purpose of explaining the invention a discharge lamp having a luminous body has been illustrated in the accompanying drawing, showing a sectional elevation of the said discharge lamp.

Referring at first to the drawing, in the axis of an evacuated glass receptacle 1 an indirectly

heated glowing cathode 2 in the form of a rod is located, which is surrounded by a screen 3 which is in the form of a funnel opening towards the apex of the glass receptacle. The said screen consists of zinc oxide and provides a conductive carrier of a surface layer 4 providing the source of light, the said layer 4 being provided on the inner side of the screen and opposite to the glowing cathode. The said surface layer 4 likewise consists of a zinc compound, and preferably it consists of zinc silicate activated by means of manganese oxide, the said surface layer 4 being made luminous by electrons emitted from the glowing cathode.

The outside of the screen 3 of zinc oxide has a metal coating 5 by means of which the current is removed.

Within the press 6 of the receptacle four wires 1, 8, 9 and 10 are fused. The metal coating 5 of the screen 3 is connected with the contact 11 through the wire 7, the cathode 2 is connected with a contact 12 through the wire 10, and the heating body 13 of the glowing cathode is connected with contacts 14, 15 through wires 8, 9. To the metal coating 5 of the screen 3 wires 16 and 17 are connected which provide a support for the screen. The wire 17 is connected to a wire 7, and it is used for removing the current from the screen.

The luminous body such as the aforesaid screen is manufactured as follows: A sintered plate of zinc oxide having a resistance of from 10 to 100 ohms per cube of one centimeter length or less and containing a few hundredths, preferably a few thousandths of a percent of manganese oxide in a state of finest distribution has a coating of colloidal silicic acid or fine silicic acid powder applied thereto, and the said plate is baked. By such baking zinc silicate containing traces of the activating manganese oxide contained in the zinc oxide is produced on the surface by transformation in solid state, the said surface emitting green light when it is impinged upon by electrons. It will be understood that in a luminous body thus manufactured the luminous substance is in large surface contact with its carrier, and that it is rigidly fixed thereto, so that the electrons are readily removed. Therefore the screens have a very high luminous density, and they emit light even if they are impinged upon by electron rays of small velocity.

In a similar way a luminous body may be manufactured on the basis of cadmium silicate phosphorus. In this case on a plate of cadmium oxide having a specific resistance of 1 ohm or less silicic

acid is spread, and it is baked so as to produce cadmium silicate.

For obtaining a particularly fine distribution of the silicate I proceed as follows: By vaporization or cathode atomization of metallic silicon on a plate of zinc oxide or cadmium oxide containing manganese a layer of silicon is produced which may have a thickness of  $1 \mu$ , preferably of from 0.1 to  $0.5 \mu$  or less. These zinc oxide plates are baked at the open air and at a temperature of more than  $400^\circ$  C., preferably at a temperature of from  $1000$  to  $1200^\circ$  C. Thereby at first silicon dioxide is produced, which thereafter forms silicates with the zinc or cadmium oxides containing manganese, so that the luminous body is produced.

The manufacture of sulfidic phosphorus may be carried out in a similar way, for example by glowing a conductive plate consisting of a mixture of cadmium oxide and zinc oxide having an addition of silver, in hydrogen sulfide at a temperature of more than  $400^\circ$  C. Thereby on the conductive carrier a luminous and very thin layer of zinc-cadmium sulfide having an addition of silver is produced which rigidly adheres to the carrier.

In a modification of the process the layers are produced as follows: To a carrier consisting of platinum or another noble metal a coating of zinc or cadmium is applied, for example by vaporization or electrolysis, or by another method, which coating is anodically transformed in an

electrolyte, or by glowing in the presence of oxygen into zinc oxide or cadmium oxide, the said oxide being treated in the manner described above. As compared to other processes, this process is a little more difficult, but it may be preferable for various purposes.

In another modification mixtures of compounds of several metals, such for example as zinc and cadmium, are subjected to the process.

I claim:

1. A luminescent body capable of light emission under excitation, comprising a conductive carrier, the surface of said carrier being luminescent and comprising a compound of a metal the same as the metal of the carrier.

2. A luminescent body capable of light emission under excitation comprising a conductive carrier of zinc oxide, the surface of said carrier containing zinc, silica, manganese, and oxygen and being luminescent.

3. A luminescent body capable of light emission under excitation comprising a conductive carrier of cadmium oxide, the surface of said carrier containing cadmium, silica, manganese and oxygen and being luminescent.

4. A luminescent body capable of light emission under excitation comprising a conductive carrier of zinc oxide and cadmium oxide, the surface of said carrier containing zinc, cadmium and sulphur and being luminescent.

WILFRIED MEYER.